

## 1

3,440,170  
PROCESS FOR THE CLEANING OF EQUIPMENT  
Jilles de Hek, Haarlem, Netherlands, assignor to  
Verenigde Kunstnijstfabrieken Mekog-Albatros  
N.V., Moliebaan, Utrecht, Netherlands, a company  
of Netherlands  
No Drawing. Filed May 28, 1965, Ser. No. 459,942  
Claims priority, application Netherlands, June 9, 1964,  
6406533; Feb. 8, 1965, 6501527  
Int. Cl. C23f 11/04; C23g 1/04  
U.S. Cl. 252—147 16 Claims

## ABSTRACT OF THE DISCLOSURE

In the cleaning of equipment constructed of metals including iron such as steel and stainless steel, an aqueous solution of an organic or inorganic acid such as citric acid or hydrochloric acid is circulated through the equipment. The solution contains a conventional corrosion inhibitor such as hexamethylene tetramine or quaternary ammonium compounds, and in addition a water soluble stannous salt such as stannous chloride. The redox potential of the solution is measured, for example, with a platinum electrode against a saturated calomel-KCl electrode, and is maintained at a value below 280 mv. by adjusting the quantity of stannous salt, whereby reduction of ferric ions to ferrous ions by steel in the equipment, and consequent corrosion, is prevented. The solution may also contain a complexing agent which forms soluble complexes with ferric ions, such as ammonium bifluoride, and which does not form soluble complexes with ferrous ions. Scale such as mill scale is dissolved without corrosion of the iron in the metal even when the solution is circulated at a high flow rate and when it is heated to elevated temperatures.

The invention relates to a process for the cleaning of equipment consisting wholly or partially of metal.

In the industry use is frequently made of equipment which, as a consequence of the medium with which it is in contact, has to be regularly cleaned. Examples of such equipment are steam boilers, pipes, reactors, heat exchangers, pumps, valves, distillation columns etc. With internal cleaning it is in some cases possible to carry out this cleaning operation by a mechanical method, such as by scaling, scraping, scouring, polishing etc. In order to carry out these mechanical operations, however, it is necessary to dismantle the equipment, whereupon the component parts may be cleaned separately.

It will be obvious that mechanical cleaning involving dismantling is time-consuming and therefore very expensive. It is also sometimes difficult and cumbersome to clean satisfactorily small spaces, which are difficult of access, such as bubble caps and rather long, in particular thin, pipes.

## 2

In view of the drawbacks involved in mechanical cleaning, attempts are being made to achieve the desired cleaning with chemical agents of such a type that the dismantling of the installation to be cleaned can be completely or substantially completely omitted. This object is achieved by the use of chemical cleaning agents which can be pumped through the equipment. This chemical cleaning method not only carries the advantage of a saving of time and labour but also improves the thoroughness of the cleaning.

The liquid cleaning agents used for this purpose are usually inorganic or organic acids. According to the nature of the contamination and of the metal to be cleaned use is made in the chemical cleaning process of inhibited or uninhibited acids, such as citric acid, sulphamic acid, phosphoric acid, nitric acid, sulphuric acid and hydrochloric acid. For this purpose the use of hydrochloric acid is usually preferred especially due to its low cost, ease of handling and great capacity for dissolving many deposits and corrosion products. An inhibitor is usually added to the acid in order to counteract as far as possible the corrosive effect of these acids on the equipment to be cleaned. Examples of such inhibitors include hexamethylene tetraamine, alkaloids and quaternary ammonium bases.

In the practical application of said chemical cleaning methods, however, serious difficulties have been encountered. When said acids are used in fact corrosion occurs—even in the presence of inhibitors—as a result of the formation of ferric ions originating from the iron-containing equipment to be cleaned and/or from the impurities containing iron compounds. This corrosion can even occur to such a large degree that after cleaning pitting and scouring are encountered in the metal of the cleaned equipment. This phenomenon occurs particularly with unalloyed steels and steels of low alloy, which are frequently used for example in steam boilers. The corrosion causes the formation of rough metal surfaces which in steam boilers lower the flow rate of the water in the evaporator tubes, with the result that a reduction of the heat transfer and an increase in the wall temperatures in the installation may occur.

When combinations of a nobler and a less noble metal are present in the equipment to be cleaned, an intensified corrosive attack on the less noble metal is found to occur. It is indeed possible to reduce this intensified corrosion, for example by blanking off or removing the nobler metal 50 of the metal combination from the apparatus before the cleaning operation, but it will be obvious that in practice this is at least inconvenient and often impracticable.

To this the following must be added. The corrosive attack appears to increase considerably when there is an 55 increase in the flow rate of the cleaning acid. Thus, when the flow rate of the cleaning acid is raised, e.g. to above 0.5 m./sec., the corrosion of the metal to be cleaned increases greatly. This means that such flow rates will have 60 to be avoided as much as possible in order to avoid

damage to the installation which is to be cleaned. This, however, may not always be possible when the equipment to be cleaned is of a complicated design. In local constrictions within a tube system for instance, excessive rates of flow may easily occur, with the result that the corrosion at such a point can assume serious dimensions.

In view of the important advantages of chemical cleaning with respect to mechanical cleaning the first-named method is used on a large scale in practice in spite of the above-mentioned drawbacks. In order, however, to keep the degree of corrosive attack to some extent within acceptable limits it is often necessary to sluice the cleaning acid one or more times during the cleaning operation, and to replace it by fresh acid. This is an attempt to keep within certain limits the content of ferric ions in the cleaning acid which are responsible for the corrosion. Even when such a measure is taken the occurrence of corrosion is in practice often unavoidable. It thus appears that, when steel comes into contact with an inhibited hydrochloric acid bath which is in motion and contains ferric compounds, at a temperature as low as 20° C., 50% of the ferric ions are reduced within 2 hours to ferrous ions at the expense of the equivalent amount of steel, which goes into solution, or in other words, corrodes. At 50° C., a normal temperature for cleaning steam boilers, for example, this degree of corrosion is reached even within an hour. Since it may take some hours to fill a fairly sizable steam boiler with cleaning fluid by means of a circulation pump, strong corrosive attack has already taken place before it is possible to proceed to sluicing the cleaning acid containing ferric ions.

It can be seen, therefore, that serious corrosion problems are invariably encountered in practice in methods of chemical cleaning of equipment by means of a cleaning acid—even when cumbersome measures are taken, like the replacement of the cleaning acid by fresh acid.

According to the present invention it has now been found that the above drawbacks can be wholly avoided if a stannous salt, which is soluble in the cleaning acid, such as stannous chloride, is added to said inhibited cleaning acid and thereby inherently forms stannous upon dissolving. When a cleaning fluid of this type is used the corrosive attack—even at high rates of flow of the cleaning acid—is found to be wholly suppressed, while if an inhibitor is used any tin which happens to be precipitated does not impair the corrosion resistance of the metal to be cleaned either.

The invention therefore relates to a process for the cleaning of equipment consisting wholly or partially of metal which comprises treating the equipment with a cleaning fluid comprising an aqueous solution of an inhibited inorganic or organic acid which, in addition, contains a stannous salt soluble in this solution.

Stannous chloride is preferably used as stannous salt soluble in the cleaning acid and therefore the source of stannous ion and inhibited hydrochloric acid as cleaning acid. Depending on the quantity and the nature of the contaminations to be removed, concentrations of the hydrochloric acid of between 0.25% by weight and 15% by weight, appear to be very satisfactory. As to the quantity of the stannous chloride, in dependence on the concentration of ferric ions in the cleaning acid, and depending upon the redox potential as will be discussed hereinbelow, quantities of between 1 and 30 g. per litre of cleaning acid which therefore corresponds to a stannous ion concentration of between 0.53 and 15.8 grams per liter of solution, are preferably used.

The advantages of the cleaning process according to the invention are many. The cumbersome and expensive sluicing of cleaning acid which contains ferric ions and is therefore corrosive—a procedure which in practice moreover is by no means always sufficiently effective

against corrosion—can now be wholly omitted. The flow rate of the cleaning acid can be raised to high values without the corrosive attack exceeding acceptable limits. In order to gain the full profit from the present invention flow rates for the cleaning acid of at least 0.2 m./sec., and preferably of between 0.5 and 3 m./sec. will be used, so that a rapid and effective cleaning can be obtained while avoiding a degree of corrosion of any substance.

The process according to the invention also provides protection against corrosive attack in equipment which contains combinations of noble and less noble metals, a protection which formerly could be only obtained by removing or blanking off the nobler metal concerned before the cleaning operation. It was thus established that by the use of the cleaning acid according to the invention the corrosive attack on the following metals or combinations of metals was wholly or substantially wholly suppressed.

|    |                                          |
|----|------------------------------------------|
| 20 | Mild steel                               |
|    | Carbon steel 50-60                       |
|    | 1% Cr-1/2% Mo-steel                      |
|    | 5% Cr-1/2% Mo-steel                      |
|    | Copper                                   |
| 25 | Brass                                    |
|    | Aluminum-brass                           |
|    | Tin-bronze                               |
|    | Cupronickel 90-10 and 70-30              |
|    | Inconel                                  |
| 30 | Nionel                                   |
|    | Nickel                                   |
|    | Monel                                    |
|    | Hastelloy                                |
|    | 13% chromium steel                       |
| 35 | 17% chromium steel                       |
|    | Stainless steel, type 18% Cr-8 to 10% Ni |

The advantages of the present invention are evidenced very clearly in the cleaning of the frequently used steels which are unalloyed or alloyed with chromium and/or nickel and/or molybdenum, in particular steels alloyed with 1-5% of chromium and 0.4-0.6% of molybdenum. In particular steel with 1% of chromium and 0.5% of molybdenum displays the phenomenon that the hydrogen which forms during the corrosive attack diffuses in the metal and gives rise to hydrogen brittleness. High pressure steam pipes are often manufactured from this material, and the disadvantage is frequently experienced with the conventional chemical cleaning methods that the corrosive attack is accompanied by hydrogen brittleness in the cleaned material, with the result that the latter easily fractures due to its brittleness. This disadvantage also is wholly obviated by using the process according to the invention.

It is also to be noted that a special aspect of the present invention is the possibility of maintaining the composition of the cleaning acid, by a simple continuous electrometric control of the cleaning fluid, at such a level that throughout the entire cleaning process the certainty exists that no corrosion, or substantially no corrosion, will occur. Thus, when measured with a platinum electrode against a saturated calomel-KCl electrode, the redox potential in the presence of a corrosive quantity of ferric ions in inhibited hydrochloric acid of 10% concentration amounts to 200 to 400 mv., depending upon the quantity of ferric ions; in the presence of a quantity of stannous ions, sufficient to counteract corrosion, the redox potential is below 280 mv. and in practice it is advisable to work below 170 mv. By means of this electrometric control it is now possible to keep the redox potential within narrow limits corresponding to a non-corrosive medium, by adjusting the desired correct composition of the cleaning acid by addition of a fresh quantity of a stannous compound.

The temperature at which the cleaning operation is carried out is usually the normal ambient temperature. In the classical chemical cleaning process it was generally necessary to avoid as much as possible temperatures higher than the ambient temperature in view of the intensified corrosive attack at elevated temperatures. The cleaning fluid used according to the invention is characterized in that also at elevated temperatures there is no corrosive attack. The upper limit of the temperature to be used is only determined by the stability of the inhibitor in the inhibited acid, and this limit generally lies around 70° C. The present invention, therefore, now provides for the first time the possibility of carrying out the cleaning operation conveniently with a cleaning fluid at an elevated temperature, i.e. at a temperature of up to 70° C.

In a preferred embodiment of the present invention a cleaning fluid is used which in addition to an inhibited inorganic or organic acid and a soluble stannous salt, contains a complexing agent specific for ferric ions. It has been found that in that case the amount of stannous salt to be used can be considerably reduced; amounts of less than 10% of the amount of stannous salt originally applied have been found to be sufficient for suppressing or substantially reducing the corrosive attack of the metal

control of the redox potential as explained above and illustrated for the combination stannous chlorideammoniumbifluoride in Example IV.

#### EXAMPLE I

5 The effect of the cleaning fluid to be used according to the invention can be seen from the data described in the following. The test results given in this example were obtained from tests which were carried out as follows.

10 Test plates from unalloyed steel (dimensions 60 x 30 x 1.5 mm.), from which plates the grease had been removed and which had been scoured bright, were exposed in duplicate in beakers containing 0.5 l. of inhibited iron-free hydrochloric acid. As inhibitor use was made of a commercially available inhibitor based on quaternary ammonium bases in a concentration of 0.2% by weight.

15 The test plates were placed vertically on their long sides in small glass racks in the beakers. Beside each exposure in a stationary medium test plates were exposed in a moving medium having a rate of 0.2 m. per second, which movement was obtained by means of an electrically powered glass stirrer. The plates were exposed for four periods, viz 8, 8, 8 and 24 hours, in the same fluid, unless otherwise stated. After each exposure the plates were weighed and examined for signs of pitting.

TABLE I  
[Medium: 10% HCl+inhibitor+10 g. of Fe<sup>+++</sup> per litre; 20° C.]

| Exposure        |      | Fluid stationary |                            |                                                      | Rate of fluid 0.2 m. per sec. |                                                        |
|-----------------|------|------------------|----------------------------|------------------------------------------------------|-------------------------------|--------------------------------------------------------|
| Period          | Hrs. | Mild steel plate | Reduction of weight in mg. | Remarks                                              | Reduction of weight in mg.    | Remarks                                                |
| 1.....          | 8    | {a.....          | 168                        | Surface slightly scoured, edges distinctly corroded. | 1,258                         | Distinct scouring particularly edges heavily corroded. |
|                 |      | {b.....          | 149                        |                                                      | 1,141                         |                                                        |
| 2.....          | 8    | {a.....          | 161                        |                                                      | 88                            |                                                        |
|                 |      | {b.....          | 162                        |                                                      | 94                            |                                                        |
| 3.....          | 8    | {a.....          | 284                        |                                                      | 34                            |                                                        |
|                 |      | {b.....          | 212                        |                                                      | 33                            |                                                        |
| 4.....          | 24   | {a.....          | 213                        | Corrosion visibly increased.....{                    | 52                            |                                                        |
|                 |      | {b.....          | 239                        |                                                      | 56                            |                                                        |
| Total over..... | 48   | {a.....          | 746                        |                                                      | 1,482                         |                                                        |
|                 |      | {b.....          | 742                        |                                                      | 1,324                         |                                                        |
|                 |      |                  |                            | Surface a=3,685 mm. <sup>2</sup>                     |                               | Surface a=3,685 mm. <sup>2</sup>                       |
|                 |      |                  |                            | Surface b=3,595 mm. <sup>2</sup>                     |                               | Surface b=3,685 mm. <sup>2</sup>                       |

TABLE II  
[Medium: 10% HCl+inhibitor+20 g. of Fe<sup>+++</sup> per litre; 20° C.]

| Exposure        |      | Fluid stationary |                            |                                             | Rate of fluid 0.2 m. per sec. |                                                               |
|-----------------|------|------------------|----------------------------|---------------------------------------------|-------------------------------|---------------------------------------------------------------|
| Period          | Hrs. | Mild steel plate | Reduction of weight in mg. | Remarks                                     | Reduction of weight in mg.    | Remarks                                                       |
| 1.....          | 8    | {a.....          | 618                        | Slight scouring, edges distinctly corroded. | 2,548                         | Rather heavy scouring of the surface; edges heavily corroded. |
|                 |      | {b.....          | 655                        |                                             | 2,227                         |                                                               |
| 2.....          | 8    | {a.....          | 432                        |                                             | 193                           |                                                               |
|                 |      | {b.....          | 429                        |                                             | 173                           |                                                               |
| 3.....          | 8    | {a.....          | 360                        |                                             | 50                            |                                                               |
|                 |      | {b.....          | 353                        |                                             | 50                            |                                                               |
| 4.....          | 24   | {a.....          | 510                        | Corrosion of the edges intensified.         | 61                            |                                                               |
|                 |      | {b.....          | 332                        |                                             | 64                            |                                                               |
| Total over..... | 48   | {a.....          | 1,920                      |                                             | 2,852                         |                                                               |
|                 |      | {b.....          | 1,769                      |                                             | 2,514                         |                                                               |
|                 |      |                  |                            | Surface a=3,745 mm. <sup>2</sup>            |                               | Surface a=3,745 mm. <sup>2</sup>                              |
|                 |      |                  |                            | Surface b=3,735 mm. <sup>2</sup>            |                               | Surface b=3,675 mm. <sup>2</sup>                              |

to be cleaned. This is more fully illustrated in Example IV.

The complexing agent should be specific for ferric ions in that it should not form a complex with the ferrous ions. This is essential for the purpose of the invention and another essential feature of the present embodiment is that an amount of the soluble stannous salt—be it a considerably reduced amount—should always be present.

Complexing agents which may be used include phosphoric acid or hydrofluoric acid or its salts of which ammoniumbifluoride ( $\text{NH}_4\text{HF}_2$ ) has been found especially suitable. The relative amounts of stannous salt and complexing agent can easily be fixed at the desired level by

When the inhibitor applied is replaced by other conventional inhibitors corresponding results were obtained, as also with the use of HCl in a 5% concentration.

65 From the above Tables I and II the following can be deduced:

(a) The corrosion increases by a factor of about 4 to 8 due to movement of the fluid at a rate of 0.2 m./sec.

70 (b) The corrosion increases greatly as the ferric-ion concentration increases, particularly in a moving medium. With exposures of 6 hours or longer, as employed in chemical cleaning i.e. in a moving medium, it can be generally stated that the corrosion due to ferric ions is proportional to the ferric-ion concentration.

It will be clear that as a consequence of the formation of pitting and scoring, the corrosion does not occur uniformly.

The effect of using stannous chloride as reducing agent is clear from the following Table III.

tions possible, viz at high flow rates of the cleaning fluid which moreover has a temperature of 50° C.

#### EXAMPLE II

##### 5 Exposure tests of (a) rotating steel discs, mild steel

TABLE III

| Exposure |      |         | A<br>(Insufficiency of Sn <sup>++</sup> ) |                                             | B<br>(Very slight excess Sn <sup>++</sup> ) |                                  |
|----------|------|---------|-------------------------------------------|---------------------------------------------|---------------------------------------------|----------------------------------|
| Period   | Hrs. | Plate   | Reduction of weight, mg.                  | Remarks                                     | Reduction of weight, mg.                    | Remarks                          |
| 1.....   | 8    | {a..... | 873                                       | Distinct scouring, edges slightly corroded. | 70                                          |                                  |
|          |      | {b..... | 870                                       |                                             | 70                                          |                                  |
| 2.....   | 8    | {a..... | 71                                        |                                             | 5                                           |                                  |
|          |      | {b..... | 71                                        |                                             | 6                                           |                                  |
| 3.....   | 8    | {a..... | 28                                        |                                             | 10                                          |                                  |
|          |      | {b..... | 34                                        |                                             | 9                                           |                                  |
| 4.....   | 24   | {a..... | 75                                        |                                             | 52                                          |                                  |
|          |      | {b..... | 76                                        |                                             | 49                                          | {No corrosion visible.           |
|          |      |         |                                           | Surface a=3,700 mm. <sup>2</sup>            |                                             | Surface a=3,520 mm. <sup>2</sup> |
|          |      |         |                                           | Surface b=3,700 mm. <sup>2</sup>            |                                             | Surface b=3,520 mm. <sup>2</sup> |

  

| Exposure |      |         | C<br>(Excess Sn <sup>++</sup> ) |                                  | D<br>(Excess Sn <sup>++</sup> ) |                                  |
|----------|------|---------|---------------------------------|----------------------------------|---------------------------------|----------------------------------|
| Period   | Hrs. | Plate   | Reduction of weight, mg.        | Remarks                          | Reduction of weight, mg.        | Remarks                          |
| 1.....   | 8    | {a..... | 72                              |                                  | 73                              |                                  |
|          |      | {b..... | 75                              |                                  | 74                              |                                  |
| 2.....   | 8    | {a..... | 3                               |                                  | 2                               |                                  |
|          |      | {b..... | 2                               |                                  | 4                               |                                  |
| 3.....   | 8    | {a..... | 2                               |                                  | 1                               |                                  |
|          |      | {b..... | 1                               |                                  | 1                               |                                  |
| 4.....   | 24   | {a..... | 4                               | {No corrosion visible.....       | 5                               | {No corrosion visible.           |
|          |      | {b..... | 6                               | Surface a=3,620 mm. <sup>2</sup> | 2                               | Surface a=3,700 mm. <sup>2</sup> |
|          |      |         |                                 | Surface b=3,670 mm. <sup>2</sup> |                                 | Surface b=3,580 mm. <sup>2</sup> |

From the above table it can be seen that stannous chloride obviates corrosion due to ferric ions almost immediately.

When an insufficiency of SnCl<sub>2</sub>, viz 6 g. of SnCl<sub>2</sub>.2H<sub>2</sub>O per litre of acid was used, corrosion still occurred in the first period of exposure.

It can also be seen from the above Table III that when

45 with mill scale; (b) welded steel pipe, mild steel, inside diameter 19 mm., through which the fluid was pumped.

Medium: 10% HCl+10 g. of Fe<sup>+++</sup> per litre+inhibitor +small excess of SnCl<sub>2</sub>.2H<sub>2</sub>O.

Temperature: 50° C. (±2° C.) for all tests.

Exposure time: 15½ hours.

TABLE IV

| Material mild steel                     | Rate of fluid with respect to the metal, in m/sec. | Exposed surface in mm. <sup>2</sup> | Reduction of weight in mg. | Reduction of weight after correction for scale in mg. | Corrosion expressed in mm./per annum | Remarks                                |
|-----------------------------------------|----------------------------------------------------|-------------------------------------|----------------------------|-------------------------------------------------------|--------------------------------------|----------------------------------------|
| a. Disc with mill scale.....            | 11.1                                               | 10,708                              | 845                        | 200                                                   | 1.3                                  | Surface entirely smooth and undamaged. |
| Do.....                                 | 12.05                                              | 10,708                              | 971                        | 325                                                   | 2.1                                  | Do.                                    |
| Do.....                                 | 13.0                                               | 10,708                              | 958                        | 312                                                   | 2.0                                  | Do.                                    |
| b. Welded pipe 400 mm. in length.....   | 2.3                                                | 23,880                              | .....                      | 654                                                   | 2.0                                  | Do.                                    |
| b. Welded pipe 2,000 mm. in length..... | 2.3                                                | .....                               | .....                      | .....                                                 | .....                                | Do.                                    |

1 Average.

20 g. or more of SnCl<sub>2</sub>.2H<sub>2</sub>O is added per litre of acid containing 10 g. of ferric ions per litre, the corrosion is negligible. The test plates were still smooth after a total time of exposure of 48 hours and contained no perceptible pitting or grooving.

When the inhibitor used in the tests shown in Table III was replaced by other conventional and commercially available inhibitors corresponding results were obtained.

The following example illustrates the use of the cleaning acid of the invention under the most adverse condi-

70 It is seen that under conditions which would lead to heavy corrosion with the known chemical cleaning methods, no or substantially no corrosion occurs.

#### EXAMPLE III

This example illustrates the cleaning of metal combinations with the process of the invention. These plates of different metals were combined with test plates of mild steel and the metal combination was exposed at 20° C. during 16 hours to cleaning acids of the composition and under the conditions set out in the following Table V.

TABLE V

10% HCl+10 g. Fe<sup>3+</sup>/l. plus inhibitor; temp. ~20° C.; rate 0.2 m./sec.10% HCl+10 g. Fe<sup>3+</sup>/l. plus inhibitor+25 g. SnCl<sub>2</sub>·2H<sub>2</sub>O/l.; temp. ~20° C.; rate 0.2 m./sec.

| Metal combination        | Red. in weight in mg. | Remarks                                                                           | Red. in weight in mg. | Remarks            |
|--------------------------|-----------------------|-----------------------------------------------------------------------------------|-----------------------|--------------------|
| Mild steel.....          | 449                   | { Steel has slight copper scale.....                                              | 3                     | { Metal unchanged. |
| Copper.....              | 76                    |                                                                                   | 2                     |                    |
| Mild steel.....          | 451                   | { Steel has no copper scale, but brass shows dark discolouration.....             | 5                     | { Do.              |
| Brass.....               | 150                   |                                                                                   | 1                     |                    |
| Mild steel.....          | 467                   | { Steel has no copper scale, but Al-brass has a black scale.....                  | 3                     | { Do.              |
| Al brass.....            | 112                   |                                                                                   | 2                     |                    |
| Mild steel.....          | 184                   | { Steel has greenish scale and Cr-steel shows dark discolouration; after scouring | 3                     | { Do.              |
| 17% Cr-steel.....        | 162                   | slight pitting visible.                                                           | 2                     |                    |
| Mild steel.....          | 205                   | { Steel has greenish scale which can be easily removed.....                       | 1                     | { Do.              |
| 18% Cr-10% Ni-steel..... | 21                    |                                                                                   |                       |                    |

It will be seen that also in the case of combinations of a noble with a less noble metal which present serious corrosion difficulties in the known chemical cleaning, corrosion is essentially suppressed when applying the process 20 of the invention.

## EXAMPLE IV

This example illustrates the use of a complexing agent specific for ferric ions as additive in the cleaning fluid 25 and the considerable saving of stannous salt obtained

Exposure of mild steel test plates in ferrous and ferric ions containing inhibited hydrochloric acid

Composition of the cleaning fluid at the beginning of the test run:

1.0 litre HCl 7.5%,

Inhibitor 0.3%,

Ammoniumbifluoride (NH<sub>4</sub>HF<sub>2</sub>), 10 grams,

Stannous chloride (SnCl<sub>2</sub>·2H<sub>2</sub>O), 1.0 gram.

Temperature 50° C.; rate of fluid 0.2 m./sec.

| Time after start of test run                                                | Addition of SnCl <sub>2</sub> ·2H <sub>2</sub> O in grams | Redox potential in mv. | Remarks                                                                                                                                                  |
|-----------------------------------------------------------------------------|-----------------------------------------------------------|------------------------|----------------------------------------------------------------------------------------------------------------------------------------------------------|
| 0 hr.....                                                                   |                                                           | -30                    |                                                                                                                                                          |
| Dissolved 10.4 g. mill scale present on mild steel plate, 1 hr. 15 min..... | 230                                                       |                        |                                                                                                                                                          |
| 7 mild steel plates placed in bath:                                         |                                                           |                        |                                                                                                                                                          |
| 1 hr. 30 min.....                                                           | 0.11                                                      | 188                    | 1. During the whole of the exposure the redox potential stayed in the range in which (in the presence of the inhibitor) no corrosive attack takes place. |
| 2 hr.....                                                                   |                                                           | 50                     |                                                                                                                                                          |
| 3 hr.....                                                                   |                                                           | 62                     |                                                                                                                                                          |
| 4 hr.....                                                                   |                                                           | 96                     |                                                                                                                                                          |
| 4 hr. 45 min.....                                                           |                                                           | 166                    | 2. The total consumption of SnCl <sub>2</sub> ·2H <sub>2</sub> O was 1.15 gram which is about 10% of the amount                                          |
| 5 hr.....                                                                   | 0.02                                                      | 96                     | required in the absence of the ferric ion complexing agent.                                                                                              |
| 6 hr.....                                                                   |                                                           | 154                    |                                                                                                                                                          |
| 7 hr.....                                                                   | 0.02                                                      | 120                    |                                                                                                                                                          |
| 8 hr.....                                                                   |                                                           | 148                    |                                                                                                                                                          |
| 23 hr.....                                                                  |                                                           | 76                     |                                                                                                                                                          |
| 24 hr.....                                                                  |                                                           | 90                     |                                                                                                                                                          |

thereby with full maintenance of the efficiency of the cleaning method according to the present invention.

Influence of fluoride on the redox potential of inhibited hydrochloric acid at varying ratios of ferrous sulphate and ferric chloride

(A) 1 litre HCl 7.5%, 0.3% inhibitor

(B) 1 litre HCl 7.5%, 0.3% inhibitor, 30 gram ammoniumbifluoride

Further additions as indicated.

Both test runs at 50° C.; rate of fluid 0.2 m./sec.

The average corrosive attack of the test plates is 0.24 mm. a year. None of the test plates showed pitting.

45 I claim:

1. In a process for the cleaning of metallic equipment constructed essentially of iron containing metal by means of a recirculating aqueous corrosion inhibited acidic cleaning solution, the improvement which comprises the steps of

(1) contacting the surface of the equipment to be cleaned with a circulating aqueous inhibited acidic cleaning solution comprising (a) from about 0.25 to

| Time              | A. Without fluoride                          |                 | B. With fluoride                             |                 |
|-------------------|----------------------------------------------|-----------------|----------------------------------------------|-----------------|
|                   | Addition in gram/litre                       | Redox potential | Addition in gram/litre                       | Redox potential |
| 0 hr.....         |                                              | 340             |                                              | 325             |
| 1 hr.....         | 5 g. ferrous                                 | 280             | 5 g. ferrous                                 | 180             |
| 1 hr. 10 min..... | 0.22 g. SnCl <sub>2</sub> ·2H <sub>2</sub> O | 40              | 0.22 g. SnCl <sub>2</sub> ·2H <sub>2</sub> O | 28              |
| 1 hr. 30 min..... | 0.2 g. ferric                                | 310             | 0.2 g. ferric                                | 65              |
| 2 hr.....         |                                              | 344             |                                              | 142             |
| 3 hr.....         | 0.1 g. ferric                                | 334             | 0.1 g. ferric                                | 236             |
| 4 hr.....         | 0.2 g. ferric                                | 338             | 0.2 g. ferric                                | 236             |
| 5 hr.....         | do                                           | 360             | do                                           | 268             |
| 5 hr. 30 min..... | do                                           | 364             | do                                           | 268             |
| 6 hr. 30 min..... | do                                           | 368             | do                                           | 280             |
| 7 hr. 30 min..... | do                                           | 370             | do                                           | 270             |

Totally added: 5 grams ferrous, 1.3 grams ferric, 0.22 gram SnCl<sub>2</sub>·2H<sub>2</sub>O, i.e. less than 10% of the amount required in the absence of fluoride to keep the fluid free from ferric ions.

The bath without fluoride is corrosive.

The bath with fluoride is non-corrosive.

75 15 weight percent of an acid selected from the group consisting of citric, sulfamic, phosphoric, nitric, sulfuric and hydrochloric acids, and (b) stannous ion in a concentration of from 0.53 to 15.8 grams per liter, the stannous ion being derived from a soluble stannous salt, and

(2) adding a soluble stannous salt to the recirculating cleaning solution in a quantity sufficient to maintain the redox potential of the solution below 280 mv. as measured by a platinum electrode against a saturated calomel-KCl electrode, whereby the ferric ion content of the solution is controlled.

2. The process of claim 1, wherein sufficient soluble stannous salt is added to maintain the redox potential below 170 mv.

3. The process of claim 1, wherein the acid is hydrochloric acid.

4. The process of claim 1, wherein the soluble stannous salt is stannous chloride and is present in a concentration of from 1 to 30 grams per liter of solution.

5. The process of claim 1, wherein the corrosion inhibitor is selected from the group consisting of hexamethylene tetramine, alkaloids, and quaternary ammonium bases and the inhibitor is present in an amount of from about 0.2 to 0.3 weight percent.

6. The process of claim 1, wherein the circulating cleaning solution has a rate of flow through the equipment of at least 0.2 meter per second.

7. The process of claim 1, wherein the circulating cleaning solution has a rate of flow through the equipment in the range of between 0.5 to 3 meters per second.

8. The process of claim 1, wherein the temperature of the cleaning solution is between ambient and 70° C.

9. The process of claim 1, wherein the equipment is constructed of a metal selected from the group consisting of steel and steel alloys with at least one of the alloyed metals selected from the group consisting of chromium, nickel and molybdenum.

10. The process of claim 9, wherein the equipment is constructed of a steel containing from about 1 to 5 percent chromium and from about 0.4 to 0.6 percent molybdenum.

11. In a process for the cleaning of metallic equipment constructed essentially of iron containing metal by means of a recirculating aqueous corrosion inhibited acidic cleaning solution, the improvement which comprises the steps of

(1) contacting the surfaces of the equipment to be cleaned with a circulating aqueous corrosion inhibited acidic cleaning solution comprising (a) from about 0.25 to 15 weight percent of an acid selected from the group consisting of citric, sulfamic, phosphoric, nitric, sulfuric and hydrochloric acids, (b) stannous ion in a concentration of from 0.053 to 15.8 grams per liter, the stannous ion being derived from a soluble stannous salt, and (c) a complexing agent for ferric ions selected from the group consisting of hydrofluoric acid and ammonium bifluoride, said complexing agent being present in an amount soluble in the acidic solution; and

(2) adding soluble stannous salt to the recirculating

5

cleaning solution in a quantity sufficient to maintain the redox potential of the solution below 280 mv. as measured by a platinum electrode against a saturated calomel-KCl electrode, whereby the ferric ion content of the solution is controlled.

12. The process of claim 11, wherein the ferric ion complexing agent is ammonium bifluoride.

13. The process of claim 11, wherein both the soluble stannous salt and the ferric ion complexing agent are added to the recirculating cleaning solution in an amount sufficient to maintain the redox potential below 170 mv.

14. The process of claim 11, wherein the redox potential is maintained at a value below about 170 mv. by the addition of stannous chloride and the ferric ion complexing agent.

15. An aqueous based cleaning composition for cleaning equipment consisting essentially of iron-containing metal consisting essentially of water, 0.25 to 15 weight percent of an acid selected from the group consisting of citric, sulfamic, phosphoric, nitric, sulfuric, and hydrochloric, from 0.053 to 15.8 grams per liter of stannous ion derived from a soluble stannous salt, from about 0.2 to 0.3 weight percent of a corrosion inhibitor selected from the group consisting of hexamethylene tetramine, alkaloids, and quaternary ammonium bases, and a ferric ion complexing agent selected from the group consisting of hydrofluoric acid and ammonium bifluoride present in an amount soluble in the cleaning solution.

16. An aqueous based cleaning composition for cleaning equipment consisting essentially of iron-containing metal consisting essentially of water, 0.25 to 15 weight percent hydrochloric acid, from 0.1 to 30 grams per liter of stannous chloride, from about 0.2 to 0.3 weight percent of a corrosion inhibitor selected from the group consisting of hexamethylene tetramine, alkaloids, and quaternary ammonium bases, and ammonium bifluoride as a ferric complexing agent in a concentration of from about 10 grams to 30 grams per liter.

40

#### References Cited

#### UNITED STATES PATENTS

|           |        |                |         |
|-----------|--------|----------------|---------|
| 1,460,395 | 7/1923 | Vogel          | 252—148 |
| 1,678,776 | 7/1928 | Gravell et al. | 252—147 |
| 1,773,247 | 8/1930 | Williams       | 252—147 |
| 2,927,871 | 3/1960 | Mancke et al.  | 156—19  |
| 3,033,795 | 5/1962 | Brevik         | 252—146 |

LEON D. ROSDOL, Primary Examiner.

W. SCHULZ, Assistant Examiner.

#### U.S. Cl. X.R.

134—3, 41; 252—87, 181